

(No Model.)

C. L. MARSHALL.  
LAMP WICK.

No. 595,884.

Patented Dec. 21, 1897.



Witnesses:

Frederick B. Hill.

Arthur d'Romatra.

INVENTOR,

Charles L. Marshall

By his attorney,

Mayron Francis Hill

# UNITED STATES PATENT OFFICE.

CHARLES L. MARSHALL, OF CEDAR GROVE, NEW JERSEY.

## LAMP-WICK.

SPECIFICATION forming part of Letters Patent No. 595,884, dated December 21, 1897.

Application filed April 3, 1897. Serial No. 630,584. (No specimens.)

*To all whom it may concern:*

Be it known that I, CHARLES L. MARSHALL, a citizen of the United States, residing at Cedar Grove, in the county of Essex and State 5 of New Jersey, have invented a new and useful Improvement in Lamp-Wicks, of which the following is a specification.

The object of my invention is to strengthen lamp-wicks which have been subjected to processes which weaken their texture though improving their lighting powers.

My invention is particularly valuable in dealing with carbonized wicks, a process for producing which is the subject of a patent 15 concurrently pending herewith. I attain this object by using in the texture of the wick some material which when subjected to the process in question will not be so affected by that process that it loses its textile 20 strength; or I may attain my object by combining with the lamp-wick material so treated new material which has not been affected by any such treatment. In other words, I aim to produce, as an article of manufacture, a 25 lamp-wick containing some strong material on which the ratchet may act, though the greater part of the wick may have been weakened by a process which is intended to improve its capillary attraction or its lighting 30 capacity.

In the process of carbonization which is the subject of the patent before referred to the fiber of the wick is necessarily weakened to some slight extent from being subjected to 35 temperatures ranging from 500° Fahrenheit to 1,200° or more. To supplement the strength of the wick in order to withstand the action of the ratchet, I introduce fibers of a substance which will not be weakened by the 40 carbonizing process. Asbestos is the substance best adapted to this purpose.

In the drawing a portion of a wick is shown, A being one of the heavy strands of the warp, and B a strand of the weft. About each 45 strand of the weft is twisted asbestos fiber C. This may be woven into the strand or twisted about it, as shown. The amount of asbestos used may be as much as sixty-five per cent. without destroying the capillarity of the wick, 50 but a much smaller amount is sufficient. Even ten per cent. will give good results.

As above noted, the material of which the wick is made may be carbonized first and the

asbestos woven in with it afterward. Thus it will be seen that there are many ways of 55 applying my idea in practice. For example, I may use a tinsel cord in the place of the asbestos.

What I do now claim, and desire to secure by Letters Patent, is—

1. As an article of manufacture, a lamp-wick composed of two sets of fibers, one set weakened by distillation and carbonization, and the other set not susceptible to such weakening.

2. As an article of manufacture, a lamp-wick having one set of fibers weakened by the abstraction of oleaginous and gummy matters and another set of fibers interwoven with said weakened fibers to strengthen them.

3. As an article of manufacture, a lamp-wick composed of interwoven carbonized and asbestos fibers.

4. As an article of manufacture, a lamp-wick having a warp and weft of carbonized 75 fibers and asbestos fibers twisted about the strands of said weft.

5. As an article of manufacture, a lamp-wick composed of a warp and weft of carbonized fibers, and asbestos fibers twisted about 80 the strands of said warp and weft.

6. The method of manufacturing lamp-wicks which consists in subjecting a wick composed of two sets of fibers, one of a refractory material and the other of a non-refractory material, to a weakening ameliorative process which acts on one of said sets of fibers and does not affect the other.

7. The method of manufacturing lamp-wicks which consists in subjecting a wick composed of two sets of fibers, one of a refractory material and the other of a non-refractory material, to a heating process which acts on one of said sets of fibers and does not affect the other.

8. The method of manufacturing lamp-wicks which consists in subjecting a wick composed of two sets of fibers, one of a refractory material and the other of a non-refractory material, to a carbonization process 100 which acts on one of said sets of fibers and does not affect the other.

CHARLES L. MARSHALL.

Witnesses:

RALPH W. HYATT,  
R. ARTHUR HELLER.